

# UNITED STATES PATENT OFFICE.

JUDSON RICE AND ANDREW STEIGER, OF SAN JOSÉ, AND ISAAC L. THURBER, OF SANTA CRUZ, CALIFORNIA.

## PROCESS OF WORKING AND USING ASPHALTUM.

SPECIFICATION forming part of Letters Patent No. 319,125, dated June 2, 1885.

Application filed October 2, 1884. (No specimens.)

*To all whom it may concern:*

Be it known that we, JUDSON RICE and ANDREW STEIGER, residing at the city of San José, county of Santa Clara, and ISAAC LANE THURBER, residing at the city of Santa Cruz, county of Santa Cruz, all in the State of California, have invented a new, useful, and Improved Process for Working and Using Asphaltum; and we do hereby declare the following to be a full, clear, and exact description of our invention.

There are large bituminous deposits in California known as "asphaltum" which is used for various purposes, but principally for roofing buildings, in paving streets and sidewalks, and for basement-floors.

The only process for working asphaltum heretofore in use has been to heat it in an open iron receptacle with coal-tar or some oily substance or ingredient, and when in a liquid state to mix it with gravel or coarse sand and subject the combination to an intense heat until thoroughly "cooked," and then to apply it in a dissolved or liquid state to the uses for which it was intended. By this process the natural qualities of the asphaltum were destroyed, the action of the fire volatilizing and evaporating portions of its valuable constituents, rendering it brittle and porous, and when exposed to the heat of the sun, or to moisture of any kind, it would crumble and decompose.

The object of our invention is to prepare asphaltum for the purposes of roofing buildings, for paving streets and sidewalks, for basement-floors, and all other purposes for which it is now commonly used by a new process heretofore unknown or used, and to preserve the natural elastic and adhesive properties contained in asphaltum in its native state without the addition of coal-tar, oil, or any other oily substance whatever, and to reduce the expense of handling it.

To carry out our invention, we take the asphaltum in its native state and soften it or dissolve it by the aid of hot water, steam, or superheated steam, and when dissolved or in a plastic state to apply it to the uses for which it is intended. We then press it with a heavy iron or rollers heated for that purpose, but not to a temperature that would burn the material, which gives it a smooth surface and renders it compact and solid.

When the asphaltum is dissolved or softened by our process, clean sand may be added, if desired, to give it the proper consistency; but without the addition of sand or other ingredient we can also use asphaltum by our process for making floor-tiling by placing the material in molds and subjecting it to pressure which gives it a firm solid form with a smooth surface which is susceptible of a fine polish.

In our process of working asphaltum we use an ordinary steam-boiler for supplying the hot water, steam, or superheated steam, and a close or open vessel, stirring by hand or by machinery.

Having fully described our invention, what we claim as new, and desire to secure by Letters Patent of the United States, is—

The process of preparing roofing and paving material consisting in the following steps: first, softening pure native asphaltum by the application of hot water or steam thereto, and, secondly, pressing it under heated rollers or other heated irons, substantially as and for the purpose set forth.

JUDSON RICE.  
ANDREW STEIGER.  
ISAAC L. THURBER.

Witnesses:

SAMUEL P. HOWES, Jr.,  
D. D. TENNYSON.